

March 23, 1937.

J. R. McELHANEY ET AL.

2,074,798

## APPARATUS FOR COATING SHEET METAL

Filed June 22, 1934



### *Inventors:*

JAMES R. McELHANEY and  
ROBERT STOKER.

by: RODERICK STOKER.  
Oliver & Ranker  
Their Attorneys.

## UNITED STATES PATENT OFFICE

2,074,798

## APPARATUS FOR COATING SHEET METAL

James R. McElhaney and Robert Stoker, Vandergrift, Pa., assignors to American Sheet and Tin Plate Company, a corporation of New Jersey

Application June 22, 1934, Serial No. 731,984

6 Claims. (Cl. 91—12.7)

This invention relates to an apparatus for coating sheet metal, and more particularly to coating such metal with tin or terne (lead and tin), although not limited thereto.

5 It is one of the objects of the present invention to smoothly and evenly coat sheet metal, as distinguished from the uneven coatings heretofore obtained, and includes the elimination of the corrugating of the metallic coating which, 10 in mill parlance, is known as "strippers."

This and further objects will be apparent after referring to the drawing, in which:

Figure 1 is a sectional elevation of the apparatus of the invention.

15 Figure 2 is a plan of the apparatus of Figure 1.

Figure 3 is a sectional view on the line III—III of Figure 1.

20 Referring more particularly to the drawing, the letter A designates a pot which is adapted to contain metallic coating compositions in a molten state.

A pair of guides 10 are disposed on one side of the pot A and have associated therewith a pair of driven guide rolls 11, which are adapted to feed 25 a sheet to be coated into a flux-box 12 which is provided with a guide plate 13 and contains the usual fluxing agents 14; such as a zinc chloride solution having an excess of hydrochloric acid. As is well known in conventional tin pot practice, 30 this fluxing agent effects a final cleansing of the surface of the sheet prior to its immersion in the molten tin or terne 15 in the pot.

A pair of feed-in guides 16 are disposed in the pot A immediately below the flux-box 12, and 35 extend downwardly to a pair of immersed feed rollers 17 which are driven in such manner as to feed the sheet between a pair of feed-out guides 18 which terminate shortly below the surface of the molten tin or terne 15 on the other side 40 of the pot A. These feed-out guides 18 are augmented by a pair of secondary guides 19 which are disposed immediately thereabove.

An oil-box 20 is disposed immediately above the upper extremities of the guides 18 and contains a suitable oil 21. A plurality of pairs of 45 driven guide rolls 22 are entirely immersed in the oil 21 immediately above the guides 19.

In conventional practice, the upper pair of these rolls 22 would only be immersed in the oil 50 in the oil-box to a point where their "nips" would be exposed to the atmosphere. This is for the reason that it is desired to squeeze the excess oil from both sides of the sheets and permit it to remain in the oil-box.

55 In tin plate practice the oil is so low in viscosity

that it "breaks" or "runs" as the sheets emerge, and but little oil adheres thereto.

In terne practice, while the oil is heavy enough to cover a major portion of the surfaces of the sheets, no attempt is made to prevent the breaking of the oil film, which is due to the low viscosity of the oil. In addition, no effort is made, in terne practice, to insure the complete solidification of the metallic coating before the oil is 5 squeezed from the sheets.

The present invention overcomes these difficulties by feeding the sheet out of the oil-box with a smooth, continuous and unbroken metal-and-oil coating thereon and maintaining the oil coating in such manner as to permit the metallic coating to solidify while thus protected. 10 This distinguishes from the prior art, wherein the majority of the oil is immediately squeezed from the sheet and it is fed to a branner, or other cleaning device. This causes the uneven 15 metallic coating of sheet metal and the production of "strippers".

In order to cool the metal-and-oil coated sheets, they are fed out of the oil-box 20 by the 20 guide rolls 22, and deflected by a guide plate 26 onto an elongated cooling table B. At the remote end of this elongated cooling table B there is disposed an oil removing means C, which is made up of a pair of squeeze rolls 30. A guard 23 extends between the housings which support 25 the ends of the guide rolls 22 and prevents foam and bubbles which are usually on the surface of the oil 21 from breaking the continuous film of oil on the sheets as they emerge from the oil-box 20. This guard 23 is in the form of a pair of 30 plates which extend between the housings and are substantially parallel to the guide rolls 22 but slightly divergent with respect to each other. The lower, and most adjacent ends, of these plates are immersed in the oil 21 immediately above and 35 proximate the submerged guide rolls 22.

The elongated cooling table B is composed of an extended collector tray 31 over which there is mounted a plurality of driven spool-shaped conveyer rolls 32, each of which is made up of a pair 45 of truncated cones with their apexes adjoining. Due to the shape of the conveyer rolls 32 the coated sheets, which are indicated at S in Figure 3, are supported on their edges only; thus preventing the breaking or roughening of the 50 oil film by contact.

As the metal-and-oil coated sheets S are moved along the cooling table B they are gradually and uniformly cooled by radiation. This permits the metallic coating to solidify in a smooth and con- 55

tinuous state. The cooling is preferably accelerated by air under pressure from nozzles 33, which are disposed along the ends of the conveyer rolls 32, air being supplied from a main 34. The disposition of these nozzles 33 is such that the air jets will be directed along the surfaces of the coated sheets S, rather than impinging thereon, which would have an agitating effect.

After the sheets S have reached the remote end 10 of the cooling table B they are assisted between the squeeze rolls 30 by a pair of guide plates 36. As the squeezed sheets S emerge from the oil removing means C they are assisted by a guide plate 37 onto a transfer means D, which is composed 15 of a driven endless belt 40 at the other end of which is disposed the usual branner or other cleaning device.

As shown in Figure 1, the collector tray 31, which is disposed beneath the conveyer rolls 32, slopes toward the oil-box 20 so as to return there- 20 to the oil removed from the metal-and-oil coated sheets S by the squeeze rolls 30. If, however, the usual palm oil were employed in the oil-box 20, it would become "cracked" from long contact 25 with the highly heated sheets and, if returned to the oil-box, would render the aggregate too viscous for use.

This condition is more noticeably evident when sheets of U. S. S. gage No. 26 and heavier are 30 processed, as they hold greater quantities of heat.

In order to obviate this difficulty, a proper viscosity of oil is maintained in the oil-box 20 despite the excess hot "cracked" oil which is re- 35 turned by the collector tray 31 from the squeeze rolls 30. This is done by making such additions to the oil-box as are necessary to compensate for permanent losses resulting from the inability of the squeeze rolls 30 to entirely remove the oil adhering to the sheets. If palm oil alone consti- 40 tuted the additions to compensate for such losses, the oil in the oil-box would gradually become so thick as to become unworkable. If a single oil is used alone as an addition it must be of a viscosity less than palm oil, or if palm oil is used there 45 must be added to it a non-mineral oil of less viscosity.

We have found that such additions should comprise a mixture of approximately 70 to 85 per cent palm oil and 15 to 30 per cent non-mineral oil (such as hydrogenated fish oil, cotton-seed oil or any non-mineral oil having a less natural viscosity than palm oil). This mixture can be added to the returned cracked oil and also to the remaining oil. The Saybolt viscosity of the oil in 55 the oil-box 20 is preferably maintained approximately about 300 to 500. If these limits of percentage of mixture and viscosity are maintained the oil will be of such consistency as to provide the proper and uniform unbroken film desired. 60 In the terne coating of said metal by our method, the mixture which is added should be composed of 78 per cent palm oil and 22 per cent non-mineral oil.

The viscosity and mixture of ingredients of 65 our oil mixture, as indicated in the preceding paragraph, are such that when replacing the oil which has been permanently lost the fresh oil combines with the "cracked" (or otherwise altered) returned oil (via collector tray 31) and the oil which remained, resulting in a mixture of 70 oils of such consistency as to provide upon the metallic coating of the sheet coming therethrough a continuous unbroken film.

We have also found that the addition of an oil 75 lower in viscosity than palm oil, either alone or

in combination therewith, results in less "cracking" or thickening than would be the case if only palm oil were used.

While we have shown and described one specific embodiment of our invention, it is to be understood that we do not wish to be limited exactly thereto, since various modifications may be made without departing from the scope of our invention, as defined in the following claims.

We claim:

1. Apparatus for coating sheet metal comprising a pot containing molten metal, an oil-box associated with said pot, means for moving a sheet through said pot and said oil-box, a cooling table extending from said pot, means for moving a sheet along said cooling table while contacting only the edges thereof, and oil-removing means associated with said cooling table, said last named means being constructed and arranged to remove the majority of oil taken up by said sheet as it moves through said oil box and return the majority of the same to the latter. 15

2. Apparatus for coating sheet metal comprising a pot containing molten metal, an oil-box associated with said pot, means for moving a sheet through said pot and said oil-box, a cooling table extending from said pot, means for moving a sheet along said cooling table while contacting only the edges thereof, a plurality of driven squeeze rolls associated with said cooling table, and means for returning the oil removed from said sheet by said squeeze rolls to said pot. 25

3. Apparatus for coating sheet metal comprising a pot containing molten metal, an oil-box associated with said pot, means for moving a sheet through said pot and said oil-box, a cooling table extending from said pot, means for moving a sheet along said cooling table while contacting only the edges thereof, means for accelerating the cooling of said sheet while on said cooling table, a plurality of driven squeeze rolls associated with said cooling table, and means for returning the oil removed from said sheet by said squeeze rolls to said pot. 35

4. Apparatus for coating sheet metal comprising, in combination, a pot containing molten metal, means for feeding the material to be coated through said pot, a box containing oil, said box being disposed adjacent and in communication with that portion of the surface of the molten metal in said pot from which said material emerges, a pair of guide rolls immersed in the oil in said box, and a pair of substantially vertically disposed plates extending from but having their lower edges immersed in said oil, the immersed edges of said plates being proximate said guide rolls. 40

5. Apparatus for coating sheet metal comprising, in combination, a pot containing molten metal, means for feeding the material to be coated through said pot, a box containing oil, said box being disposed adjacent and in communication with that portion of the surface of the molten metal in said pot from which said material emerges, a pair of guide rolls immersed in the oil in said box, a pair of substantially vertically disposed plates extending from but having their lower edges immersed in said oil, the immersed edges of said plates being proximate said guide rolls, a transfer table extending from said box, and a plurality of driven squeeze rolls associated with said transfer table. 60

6. Apparatus for coating sheet metal comprising, in combination, a pot containing molten metal, means for feeding the material to be 65

coated through said pot, a box containing oil, said box being disposed adjacent and in communication with that portion of the surface of the molten metal in said pot from which said material emerges, a pair of guide rolls immersed in the oil in said box, a pair of substantially vertically disposed plates extending from but having their lower edges immersed in said oil, the

immersed edges of said plates being proximate said guide rolls, a transfer table extending from said box, coolant dispensing means on said transfer table, and a plurality of driven squeeze rolls associated with said transfer table.

5

JAMES R. McELHANEY.  
ROBERT STOKER.